

Aug. 29, 1933.

C. A. DALEY

1,924,846

METHOD OF TREATING RAILROAD TRACK MEMBERS

Filed May 8, 1931

*Fig. 1.*



*Fig. 2.*



INVENTOR  
*Charles A. Daley*  
BY  
*J. H. Landenbury*  
ATTORNEY

## UNITED STATES PATENT OFFICE

1,924,846

METHOD OF TREATING RAILROAD TRACK  
MEMBERSCharles A. Daley, Hornell, N. Y., assignor to Air  
Reduction Company, Incorporated, New York,  
N. Y., a corporation of New York

Application May 8, 1931. Serial No. 535,863

2 Claims. (Cl. 148—21.5)

It has long been a problem with railroad engineers to find some method or means of preventing so-called "batter" at the ends of the rails, that is to say, at the joints, in railroad tracks.

In order to prevent or reduce this wear, it has been proposed to harden the tread portions of the rails, for a short distance from each end and to a moderate depth, by locally heating these regions above the point of decalescence by means of the oxyacetylene flame, and thereupon quenching the rail ends with water. In the course of study and experiment in connection with this track problem I have found that such a treatment defeats its purpose, since strains are set up which cause the treated portions of the rail to chip and spall, producing a condition worse than the normal wear.

The wearing down of rail ends is to a large extent due to the cold flow of the metal caused by load on the rails exceeding the elastic limit. When trains pass over a rail the concentrated load applied under the wheels produces at times a stress greater than the elastic limit of the steel in the rail. At any point between the ends of the rail this would tend to produce a permanent deformation were it not that the metal at the bearing point is always backed up by a mass of metal at both sides. At the ends of the rail the effect of cold flow becomes in time very noticeable, and its results are not only a lowering of the surface but also a breaking away of material from the tread ends due to the liping over of the metal and the working of these lips against each other as the ends move up and down.

The object of this invention therefore, is to raise the elastic limit of the tread portions of the rails or other track members, at and adjacent their ends, sufficiently to overcome or greatly reduce the cold flow effect, thereby minimizing "batter" and materially prolonging the life of the rails, while at the same time purposely avoiding the production of any high degree of hardness. It will be understood that the elastic limit of the metal can not be raised without increasing the hardness, but in my process of treating rail ends hardness is a concomitant rather than the objective and is rigorously limited.

By playing the flame of the oxyacetylene torch on the end portions of the tread surface until a tread surface layer is heated locally well above the transformation range, quenching the rail ends under proper control, and then drawing the temper, I find that I can raise the elastic limit of the steel to an extent giving very useful re-

sults without danger of causing the rail ends to crack or spall. For rails of ordinary composition (carbon about 0.70%—0.85%) it is important that the heat treatment of the tread surfaces of the ends of the track members be not allowed to result in a hardness much above a Rockwell hardness of C40—C45. By conducting the operation so as to produce a superficial hardness of approximately this value, the elastic limit of the metal in the treated regions is raised sufficiently to stop or very greatly retard the flow of metal at the ends of the rails, and with entire safety that the rail ends will not develop failure as the result of the heat-treatment. The conditions of the control are variable and can scarcely be specified but will be readily practiced by those skilled in the art when the object to be attained and the permissible degree of hardening is kept in mind.

The heat treatment of the top of the rail end is to be accomplished quickly, so as to avoid altering the structure of the body of the rail end, for which reason the oxyacetylene flame played on top of the rail ends is particularly effective, but other means of heating may be employed. The tread surface of the rails is heated above the point of decalescence to a depth of about one-quarter of an inch and for a distance of a few inches back of the adjoining or approximate ends of the rails, and as soon as this is accomplished the heated regions are quenched with water down to about 300° F. and then re-heated to about 650° F. This re-application of heat, by which the treated regions are reheated to a much lower temperature than before is necessary in order to draw the temper at the very end of the top surface of the rail, without which chipping would result.

Rail ends are so treated in accordance with this process as to wear down practically uniformly with the untreated, major portions of the rail. Rail batter being the amount of depression of the running surface at the ends as compared with the remaining running surface of the rail, it follows that if the whole length of the rail wears down uniformly no batter will exist. It is a purpose of this invention to raise the elasticity and hardness of the metal of the tread at the rail ends just sufficiently to retard the cold flow at these regions and to enable them to resist the hammer blows of the car and engine wheels passing from one rail to the other, to an extent which keeps the ends of the rail from wearing down more rapidly than the tread of the main part of the rail.

In the accompanying drawing:

Fig. 1 is a side elevation of the ends of two rails at a joint in the track; and

Fig. 2 is an end elevation of one of the rails, the views indicating schematically by dotted and shade lines the approximate extent and depth of the treated areas.

In these views the rails are marked 2, and the heat-treated regions are marked 3.

It is contemplated that the rails will be subjected to the treatment while in place in the track, but the rail ends may be given the treatment before they are laid or at the mill where they are produced.

The method is equally applicable in connection with the building up of worn rail ends by depositing metal under fusion on the worn ends, as by means of the oxyacetylene torch and welding rod. In such event, the treatment would be applied to the rail ends after having been re-  
20 stored in this manner.

It will be understood that rail steels of different compositions will require somewhat different control of time, temperature and volume of cooling medium, and that different sizes of rails  
25 will also require somewhat different control, these matters being within the skill of the operator. When worn rails are built up, the precise conditions of control in the treatment of the built-up rail ends will also depend to some extent on the  
30 composition of the metal which has been added.

It is an advantage of that application of the invention that wear-resisting built-up rail ends can be obtained without using alloy rods of special composition designed to form a wear-resisting surface. It will be understood, therefore, that the invention is not limited to precise temperatures, since the optimum temperatures will necessarily depend upon the particular compositions of the rails and the service to which they are put.

I claim:

1. A method of treating the ends of railroad rails in the track which comprises quickly heating the upper tread portions of the same above the critical range of the steel, at and adjacent the ends only, quenching the heated regions to about 300° F., and then reapplying heat to the said portions so that they are reheated to about 650° F., substantially as and for the purpose set forth.

2. A method of treating the ends of railroad rails in the track, which comprises quickly heating the upper tread portions of the same above the critical range of the steel, at and adjacent the ends only, by local application of a torch flame, quenching the heated regions to about 300° F., and then reapplying the torch flame to the said portions so that they are reheated to about 650° F., substantially as and for the purpose set forth.

CHARLES A. DALEY. 105

35

110

40

115

45

120

50

125

55

130

60

135

65

140

70

145

75

150